

C. W. ADAMS, JR.  
SINTERING IGNITION PROCESS.  
APPLICATION FILED JAN. 19, 1917.

1,299,892.

Patented Apr. 8, 1919.

2 SHEETS—SHEET 1.



**WITNESS**

W. F. Green of Worcester

**INVENTOR**

INVENTOR  
Charles W. Adams Jr.  
BY Messmer & Austin  
ATTORNEYS

C. W. ADAMS, JR.  
SINTERING IGNITION PROCESS.  
APPLICATION FILED JAN. 19, 1917.

1,299,892.

Patented Apr. 8, 1919.  
2 SHEETS—SHEET 2.



WITNESS

*John W. Adams*

Charles W. Adams, Jr. <sup>INVENTOR</sup>  
BY *Messimer + Austin*  
ATTORNEY

# UNITED STATES PATENT OFFICE.

CHARLES W. ADAMS, JR., OF MURRAY, UTAH, ASSIGNOR TO AMERICAN SMELTING & REFINING CO., A CORPORATION OF NEW JERSEY.

## SINTERING IGNITION PROCESS.

1,299,892.

Specification of Letters Patent.

Patented Apr. 8, 1919.

Application filed January 19, 1917. Serial No. 143,236.

To all whom it may concern:

Be it known that I, CHARLES W. ADAMS, Jr., a citizen of the United States, and resident of Murray, in the county of Salt Lake 5 and State of Utah, have invented certain new and useful Improvements in Sintering Ignition Processes, of which the following is a specification.

My invention relates in general to an improvement in the process of roasting and sintering metalliferous ores and particularly relates to an improvement in the steps incidental to that part of the process which relates to the igniting of the charge of ore. 10 One method of sintering ores as at present practised is to deposit a layer of the ore on the upper run of an endless series of grates or pallets which carry the layer of ore under some form of igniting device and over one or more wind or suction boxes 15 arranged to draw air downwardly through the igniting charge. The depth of the layer of ore and the speed of the pallets across the wind boxes are so proportioned that 20 the ore is roasted and sintered by the time the ore has reached the end of its travel.

Numerous forms of igniting devices have heretofore been used. A small coal burning furnace has been used with some success 25 but a furnace using some kind of hydrocarbon fluid such as gasoline, oil or gas has so far proved to be the most satisfactory. While these hydro-carbon furnaces are entirely satisfactory in igniting certain classes 30 of ores, when used with other classes of ores they are seriously objectionable, among other reasons because the process as practised with these furnaces entail serious metal losses especially in the lead and silver metals.

Further it appears that when these hydro-carbon burning furnaces are used with certain ores the intense ignition incidental to their use causes a glazed or fused crust to form on the ore during the initial part of 40 the sintering operation and this crust makes the charge semi-impermeable to the passage of the air so that an amount of oxygen is drawn through the charge insufficient to complete the formation of the compounds 45 containing  $SO_2$  and  $SO_3$  radicals. The result is that the sulfur in elemental form is carried into the flues and passageways. Under temperature conditions suitable there-

for, this elemental sulfur ignites, causing rapid expansion of the gases. A condition 55 similar to an explosion takes place which interferes with the successful operation of the process.

Accordingly, one of the objects of this invention is to improve the usual method of 60 sintering, particularly in the igniting features thereof, so that the metal losses may be reduced to a minimum, and, incidentally to this feature, to eliminate the serious danger 65 from the igniting of elemental sulfur in the flues.

A further object of the invention is to provide a simple and inexpensive process by means of which the ore may be ignited economically and to provide a process susceptible 70 of such control that the mass of igniting material fed per unit of ore mass may be varied readily to suit the requisites of the particular ore under treatment.

One method of obtaining these objects is to 75 ignite the charge of ore quietly after it has been placed on the traveling pallets and to effect the ignition without the intensity of igniting action characterizing the active flame form of ignition heretofore used in 80 operations of this character. With the present installation of one known form of sintering machine, this action is most satisfactorily effected by depositing a thin layer of 85 a flameless body such as a hot roasted ore on the spread charge of ore to be roasted just before the charge with its hot top layer is passed over the vacuum boxes. A thin layer of hot sulfid ore calcines having a 12 to 15 per cent. sulfur content has been used 90 with much satisfaction in a plant where such an ore is available but it is to be understood that this particular ore is merely suggestive of one type of ore suitable for the purpose and practically any semi-roasted ore or 95 other hot product available about a smelting plant may be utilized to effect the igniting feature of this invention.

As a matter of economy in handling and 100 to maintain a fairly high igniting temperature, the hot ore is fed preferably from a furnace arranged with its outlet close to the layer of ore to be sintered and in advance of the vacuum or wind boxes. As the layers are passed over the vacuum boxes the igniting layer brightens up and the lower line 105

of the burning zone travels slowly and quietly down through the ore thus completely sintering the charge.

The process has been carried out with advantage by means of a sintering machine of the conveyer type such as illustrated in the accompanying drawings in which—

Figure 1 is a side elevation of one end of a Dwight and Lloyd sintering machine 10 shown in connection with an ore supplying furnace and

Fig. 2 is a transverse sectional view taken on the line 2—2 of Fig. 1.

The machine illustrated is the charging end of a straight line sintering machine including a supporting frame 3 which supports an endless chain of grates or pallets 4 passing about and actuated by some suitable driving means such as a sprocket wheel 5. A feed hopper 6 is positioned to direct a continuous stream of the ore to be treated on to the upper run of grates and to spread the same evenly in a layer of uniform thickness. The most satisfactory working thickness of this layer is dependent obviously upon the capacity of the machine, the rate of travel of the grates and the character of the ore under treatment, but in general, working with a layer of four to six inches has given 30 the most satisfactory results.

The igniting device illustrated includes a small mechanical roasting furnace 7 having a discharge outlet 8 for the hot ore 9 and a depending hopper 10 leading down from 35 the furnace outlet and terminating in a discharge nozzle 11 arranged to spread the hot ore from the furnace in a thin layer on top of the charge of ore to be roasted. The discharge nozzle of the hopper or chute 10 is in 40 the form of an adjustable gate arranged to control the depth of layer of hot ore discharged from the chute on to the ore to be roasted. In the device illustrated this adjustable nozzle is in the form of a long narrow band telescoping the lower end of the chute and adjustable in its vertical position by means of the hand wheel 12 acting through the pinions 13 on a hand wheel shaft 14 meshing with racks 15 projecting 45 upwardly from the nozzle. Positioned beyond the ore discharging chute is a plurality of vacuum or wind boxes 16 a part of one of which is shown in the drawings.

These wind boxes are designed to cause a 55 downwardly directed draft of air to pass through the top hot layer of ore and through the charge of ore to be sintered as is usual with devices of this character.

In operation it will be understood that the 60 charge of ore to be treated is spread evenly on the grates as is usual with machines of this character using other forms of igniting devices. A layer of hot ore from the roasting furnace is then spread evenly on top of 65 the spread charge to be sintered, the depth

of the layer of hot ore best suited for a successful ignition depending upon the character of charge to be ignited, upon the rate of travel of the grates across the wind boxes and, to some extent, upon the temperature 70 of the hot ore deposited in the charge to be sintered. With one type of charge a layer of about one-half inch of hot ore at a bright red heat has been used with much satisfaction.

This flameless method of igniting the sintering charge has eliminated several objectionable features of the usual hydro-carbon flame method as heretofore used and has produced results and advantages which has 80 improved the process from a commercial standpoint. The metal losses which have heretofore amounted to a considerable percentage of the charge have been reduced materially so that these losses with the improved igniting are now almost negligible. 85

The sulfur present in the charge appears to be completely oxidized so that little, if any, elemental sulfur passes into the flues. This feature has resulted in a material saving 90 in cost of the flue construction in that the safety valves and other devices for preventing explosions in the flue can now be eliminated. This new method also eliminates the possibility of danger resulting from the 95 handling of liquid fuel in the old form of igniters and also eliminates the cost of this liquid fuel which recently has added materially to the cost of the sintering operation.

Further, this new process is valuable in, 100 that the finished product is more thoroughly sintered than by the over ignition to which the charge has heretofore been subjected and this perfected sintering is obtained at a materially less cost per ton of charge treated. 105

I claim:

1. In the art of sintering ores, the process which consists in spreading a uniformly thick layer of red hot ore in direct physical contact with the top of a charge of the ore 110 to be sintered and subjecting the layer and charge to the action of a downwardly directed current of air passed through the same.

2. In the art of sintering ores, the process 115 which consists in subjecting the ore to be sintered to the action of a body of hot ore in contact therewith and passing a current of air through the ore to be sintered and in a direction away from the body of hot ore. 120

3. In the art of sintering ores containing sulfur, the process which consists in covering a charge of the ore calcines containing sulfur to be sintered with a layer of hot ore adapted to prevent the formation of a glazed 125 or fused top crust to the charge during the sintering of the charge and sintering the ore so covered.

4. In the art of sintering ore containing sulfur, the process which consists in deposit- 130

ing on top of a layer of the ore, a layer of red hot ore having a temperature sufficiently high to quietly ignite the charge and at a temperature sufficiently low so as to distil only a relatively small amount of elemental sulfur from the ore and subjecting the ignited ore to a down draft of air.

Signed at Murray, in the county of Salt Lake, and State of Utah, this 14th day of December A. D. 1916.

CHARLES W. ADAMS, JR.

Witnesses:

A. H. RICHARDS,  
W. W. NORTON.